

## UNITED STATES PATENT OFFICE.

RAOUL ADRIEN GRIMOIN-SANSON, OF PARIS, FRANCE.

## TREATMENT OF CORK FOR THE MANUFACTURE OF CORK FABRIC.

SPECIFICATION forming part of Letters Patent No. 779,277, dated January 3, 1905.

Application filed July 30, 1904. Serial No. 218,915.

*To all whom it may concern:*

Be it known that I, RAOUL ADRIEN GRIMOIN-SANSON, a citizen of the Republic of France, and a resident of Paris, France, have invented 5 a new and useful Improvement Relating to the Treatment of Cork for the Manufacture of Cork Fabrics, which improvements are fully set forth in the following specification.

Cork has frequently hitherto been employed 10 in combination with fabrics for the purpose of obtaining a light and impermeable product, which has found numerous applications in hat-making, the manufacture of clothing, and the like. These cork fabrics are generally prepared 15 by fixing thin strips of cork to the fabric either by means of a suitable cement or by uniting the two by pressing them together under heavy pressure. It has been found that the latter method cannot be successfully effected; and the present process has for its object 20 certain improvements in the method of uniting the cork and fabric by cement in such a way that the resulting product is fully as supple as that prepared by the method in which 25 pressure is employed, and possesses the advantage that the parts are efficiently united, a result which it is impossible to effect by means of pressure.

The novel process is carried out in the following manner: After having triturated the 30 cork which it is intended to treat the small pieces are subjected to pressure in any suitable press, so that a block of convenient size is formed. This block is subjected to a temperature of 120° centigrade for approximately 35 three hours, so as to effect the more intimate connection between the small constituent particles, the block being then placed in a suitable cutting-machine and cut into sheets of 40 about one-tenth of a millimeter in thickness. In this form of exceedingly thin sheets the cork is then submitted to a chemical treatment, serving to remove from the cork the 45 portions which render it liable to break. The procedure is as follows: In a large boiler capable of withstanding a pressure of six atmospheres and capable of containing about 50 three hundred liters are poured ordinary benzin, eighty liters; essence of turpentine or carbon sulfid, eighty liters; ordinary glycerin,

three liters; Para rubber, five hundred grams; hydrochloric acid, five thousand grams. After the mixture has been well agitated and rendered homogeneous the thin sheets of cork are placed therein and the whole is submitted 55 to a temperature of 65° centigrade for about two hours and a half. After this treatment the sheets need not be dried. They may at once be used for the reception of fabrics or tissues of any kind. The application of fabrics, leather, canvas, or other material to the sheets of cork prepared in this way is effected in the following manner: The material is first of all freed from all dust which might prejudicially affect the perfect adhesion of the sheets 60 of cork to it. It is then stretched upon a tentering-roller, which conducts it beneath the roller distributing the substance serving to fix the cork to the fabric. This agglutinant solution is composed in the following manner: petroleum-ether, ten liters; ordinary caoutchouc, one kilogram; acetone, fifty grams. Before employing this solution it is allowed to macerate for forty-eight hours in order to facilitate 65 the solution of the caoutchouc. The sheets of 70 cork prepared in the manner described above are arranged side by side by an automatic distributor which arranges them upon the fabric provided with the agglutinant solution. Then in order that the adherence may be perfect 75 the cork-coated material is passed between three rollers, the pressures of which increase progressively. The product obtained then passes into a stove, heated to 60° centigrade, upon copper rollers heated by steam and finally 80 into a ventilated stove, where the drying is completed and in which the odor of the products employed disappears completely. Finishing or retouching is then effected, if necessary.

Cork which has undergone the treatment 85 described for eliminating the friable portions may be united with fabrics of any kind, presenting either a large or small mesh, also with leather and other materials, and these combinations may be for applications of all kinds. 90

I claim—

1. The process of manufacturing cork fabric, which consists in forming the cork into thin sheets, treating the same with a mixture of benzin, turpentine or carbon sulfid, glycer- 100

in, Para rubber and hydrochloric acid in order to separate the friable portions therefrom, and then suitably applying said sheets to a fabric.

2. The process of manufacturing cork fabric, which consists in forming the cork into thin sheets, immersing the same in a mixture of benzin, turpentine or carbon sulfid, glycerin, Para rubber and hydrochloric acid, submitting the whole to a temperature of approximately  $65^{\circ}$  centigrade, removing the sheets from said mixture, and suitably applying said sheets to a fabric.

3. The process of manufacturing cork fabric, which consists in forming the cork into thin sheets and fixing said sheets to a suitable fabric by means of a paste composed of petroleum-ether, caoutchouc, and acetone.

4. The process of manufacturing cork fab-

ric, which consists in forming the cork into thin sheets, removing the friable portions therefrom, and then fixing said sheets to a suitable fabric by means of a paste composed of petroleum-ether, caoutchouc, and acetone.

5. A cork fabric, comprising a thin sheet of cork from which the friable portions have been removed, and a sheet of fabric united therewith by means of a paste composed of petroleum-ether, caoutchouc and acetone.

In testimony whereof I have signed this specification in the presence of two subscribing witnesses.

RAOUL ADRIEN GRIMOIN-SANSON.

Witnesses:

EMILE LEDRES,  
HANSON C. COXE.